

## UNITED STATES PATENT OFFICE

GEORGE A. RICHTER, OF BERLIN, NEW HAMPSHIRE, ASSIGNOR TO BROWN COMPANY, OF BERLIN, NEW HAMPSHIRE, A CORPORATION OF MAINE

## PROCESS OF CONDITIONING CELLULOSIC FIBER FOR THE MANUFACTURE OF RAYON

No Drawing. Application filed July 13, 1926, Serial No. 122,271. Renewed June 28, 1929.

This invention relates to the conditioning of cellulosic fiber for the manufacture of rayon by the viscose process, and has for its object to make available as a satisfactory raw material for rayon manufacture, without change of present equipment, certain cellulosic fibers with which difficulty is encountered if treated in accordance with the usual commercial methods.

- 10 In preparing rayon, it is now common practice to purchase as a raw material un-beaten pulp in sheet form. The sheets are submerged in a bath of caustic soda of the proper concentration and are soaked while 15 suspended either vertically or horizontally until thoroughly saturated with the solution. The saturated sheets are removed from the bath and any excess solution is removed from the sheets by pressure. The sheets are then 20 shredded or disintegrated into fiber flocks, which are allowed to age or condition for a suitable period and are finally converted into viscose or cellulose xanthate by treatment with carbon bisulphide.
- 25 The handling and treatment of pulp while in sheet form with a caustic soda solution are simple and economical, but it is desirable that the pulp be retained in sheet form during treatment, to permit it to be removed 30 and finally pressed as such, as this facilitates handling of the material. The usual commercial unbeaten sulphite pulp, cotton fiber, or refined sulphite pulp high in alpha cellulose content, when submerged in caustic soda 35 solution in the form of sheets, retains such form satisfactorily and no difficulty is encountered in this treatment, but nevertheless such raw material, due to inequality of fiber size and other factors, requires a prolonged 40 depolymerization reaction period for complete conversion of its largest fibers into alkali cellulose, and results in a non-uniform reaction and an undesirable degradation of the shortest fibers, which undergo further 45 changes in the period required for such complete conversion of the largest fibers. On the other hand, when sheets of unbeaten kraft pulp are submerged in a caustic soda solution, they become soft and punky, and soon dis- 50 integrate. This leads to inconvenience and

difficulty in removing the pulp from the bath and its subsequent handling.

I have found that if kraft or soda or other pulp is first beaten to a material extent and then formed into sheets, disintegration will 55 not take place when such sheets are submerged in a caustic soda solution preparatory to conversion into viscose and a much more uniformly treated product, which depolymerizes more uniformly and which gives 60 a higher yield of a better quality viscose, is realized. In accordance with this finding, therefore, the pulp is beaten or hydrated to a moderate or greater slowness, and is then formed into waterleaf sheet or paper on a 65 paper machine. The beaten, sheeted pulp may be soaked in a caustic soda solution of proper concentration until it has absorbed sufficient caustic soda for subsequent treatment without undergoing disintegration, and 70 may be removed and subjected to pressure while in sheet form for the removal of excess solution. After ageing the sheeted pulp under the proper conditions for the necessary period, it may be shredded into fiber 75 flocks and then xanthated.

It is my opinion that when an unbeaten kraft sheet is treated with a caustic soda solution prior to xanthation, sufficient ligneous matter and pentosan is dissolved and removed 80 from the interfelted fibers to cause a general softening and loosening of the fibers and consequent disintegration of the sheet. This disintegrating action on kraft sheets may be imputed to the fact that kraft digestion leaves 85 a higher percentage of ligneous matter and pentosan in the resulting pulp than sulphite digestion, which is especially effective in dissolving and removing such constituent. If the pulp is beaten or hydrated to a sufficient 90 slowness prior to sheeting, however, a sufficiently tenacious bonding or cementing together of the interfelted fibers is effected to retard or resist disintegrating action in 95 a strong caustic soda solution.

In instances where pulp of other variety, such as soda pulp derived from spruce, pine, birch or poplar, or kraft or soda pulps which have been bleached, or refined by further 100 alkaline treatment, as described in my ap-

lication Serial No. 73,193, filed December 4, 1925, undergoes disintegration when treated in sheet form with a caustic solution prior to xanthation, such disintegration is prevented, in accordance with the present invention, by beating the pulp to a sufficient extent prior to its sheeting and subsequent treatment with caustic soda solution.

In the treatment of pulp such as herein referred to for xanthation purposes, it is found that a substantial beating of the pulp and its formation into waterleaf paper produces other highly desirable results. Thus, beating effects a greater uniformity of fiber size and 10 a greater uniformity of fiber distribution, and consequently a sheet of paper of uniform thickness and texture is secured. As a result, a more uniform impregnation of the fibers with caustic soda in the first step of 15 the viscose conversion process is effected. Similarly, in ageing or seasoning the sheets, a more uniform depolymerization of the fibers is effected, and when such sheets are shredded, more uniform fiber flocks are produced, which xanthate more uniformly and 20 in a shorter period of time without leaving such a high proportion of unxanthated fibers or so-called "whiskers," which are liable to clog the orifices of the spinnerets and which 25 must, therefore, be filtered out.

I do not herein claim the subject matter of patent application, Serial No. 97,998, filed March 27, 1926, by Milton O. Schur, Royal H. Rasch, and myself, wherein the advantages 30 of beating cellulose fiber prior to nitration are disclosed, or the subject matter of its continuation application, Serial No. 140,674, filed October 9, 1926. Nor do I herein claim broadly the subject matter of my application, 35 Serial No. 194,506, filed May 26, 1927, which discloses the advantages of first preparing a waterleaf paper from cellulose fiber, and then xanthating such paper. Nor do I herein claim broadly the subject matter of my application, 40 Serial No. 196,135, filed June 2, 1927, which discloses the advantages of materially reducing or pulverizing cellulose fiber prior to conversion into derivatives such as cellulose xanthate.

45 Having thus described this invention, it should be obvious that it is susceptible of various changes and modifications without departing from its spirit or scope as defined by the appended claims.

50 What I claim is:

1. A process which comprises beating a pulp which undergoes disintegration if soaked in unbeaten sheet form in a solution of caustic soda, sheeting the beaten pulp, treating the sheeted pulp with caustic soda solution, and converting the treated sheet into viscose.

2. A process which comprises beating pulp derived from alkaline digestion, sheeting the pulp, treating the sheeted pulp with a solu-

tion of caustic soda, and then converting the treated sheets into viscose.

3. A process which comprises beating a pulp derived from alkaline digestion, forming such pulp into waterleaf sheet, submerging the sheet in a solution of caustic soda, removing such sheet from the solution, expelling excess solution therefrom, and converting the sheet into viscose.

4. A process which comprises beating a pulp derived from alkaline digestion, forming the pulp into a waterleaf paper, treating the paper with caustic soda solution, and converting the treated paper into viscose.

5. A process which comprises beating cellulose pulp, converting the beaten pulp into sheet form, immersing the sheet in caustic soda solution, shredding the sheet, and xanthating the shreds.

In testimony whereof I have affixed my signature.

GEORGE A. RICHTER.

70

75

80

85

90

95

100

105

110

115

120

125

130